

2,236,899

April 1, 1941.

E. FETZ

ALLOY

Filed Feb. 17, 1939



## UNITED STATES PATENT OFFICE

2,236,899

## ALLOY

Erich Fetz, Newark, N. J., assignor to Wilbur B.  
Driver Co., Newark, N. J., a corporation of New  
Jersey

Application February 17, 1939, Serial No. 256,966

4 Claims. (Cl. 75—171)

The invention relates to alloys and more particularly to improvements in the life characteristics of alloys adapted for electrical resistance uses.

In my co-pending application, Serial No. 231,597, entitled "Alloy," I have disclosed a product consisting essentially of nickel and chromium, or, nickel, chromium and iron, with either of which basic alloys boron is compounded for the purpose of improving the hot workability of the resultant metal.

This invention has for its principal object the improvement of the life characteristics of alloys of the type disclosed in my beforementioned application.

It is yet another object of the invention to attain desirable life characteristics in alloys of the beforementioned class without an attendant decrease in the workability or forgeability of the resultant product.

A more specific object of the invention resides in the provision of an alloy of relatively longer life characteristic than has heretofore been attainable without detracting from the commercial utility of the product.

It is a well established hypothesis in the art that the life of resistance alloys such, for example, as nickel-chromium, and nickel-chromium-iron, when submitted to high temperatures, is a function to a large extent of the crystalline structure of the product. This physical characteristic of the alloy is greatly influenced by the high affinity of chromium for oxygen, nitrogen and carbon at the high melting temperatures employed in the manufacturing operation. The molten metal is contaminated by the formation of oxides, nitrides, carbides, etc., which accumulate at the crystal boundaries upon solidification. When the alloy is subsequently raised to the operating temperatures common to resistance wire applications, these non-metallic accumulations at the crystal, or grain boundaries, are presumed to react differently from the pure metal due to their different co-efficients of expansion, with the result that further oxidation occurs between the bodies of the crystals themselves until the wire, or such other form as the resistance element may take, fails physically.

It has accordingly been the practice to add such substances as silicon, aluminum, calcium, magnesium, beryllium, zirconium, cerium, etc., to the basic alloy with a view to removing the non-metallic impurities introduced during the melting process, as well as to increase the oxidation re-

sistance of the finished product at service temperatures.

In the United States Patent to Hunter No. 2,005,423, for example, it was proposed that calcium be added to a basic nickel-chromium alloy in quantities ranging from 0.03 to 0.2% to improve the life characteristics of the finished product. Similarly, in the patents to Lohr, Nos. 2,005,430, 2,005,431, 2,005,433, and 2,047,916, the beneficial effects of additions of such elements as molybdenum, zirconium and calcium to basic nickel and chromium, or, nickel-chromium-iron alloys is clearly pointed out.

I have found, however, that the presence of any one or more of these oxidation resisting diluents impairs the hot workability of the product and that any effort to attain ideal life characteristics by increasing the percentage of diluent employed renders the product altogether unforgeable and, thus, commercially useless.

For example, a series of melts were made in which 150, 160, 175, 190 and finally 250 grams of calcium silicon were added to the basic alloy of nickel and chromium. The alloys containing 150 and 160 grams respectively of calcium silicon showed poor results in forging tests, while those alloys containing the relatively higher percentages of calcium silicon were altogether unforgeable. Thus, it will be apparent that the percentage of the life imparting diluents which may be employed in any given alloy is a function of, and limited by, the ability to work the finished product.

I have found that the addition of boron to the basic alloy permits of the use of greater percentages of the life imparting diluents without adversely affecting the forgeability of the finished alloy.

To illustrate the effect of the presence of boron upon the total percentage of a life imparting diluent which may be added to the basic alloy without destroying its forgeability characteristics, I have prepared nickel-chromium alloys containing the identical quantities of calcium silicon set forth in the above enumerated tests with the addition in each instance of 50 grams of manganese boron.

For the purpose of determining the life of these alloys at high temperatures, I have tested that series which contained boron by the method of test outlined in American Society for Testing Materials, Designation B76-36, Book of A. S. T. M. Standards, 1936, page 734.

*Test specimen*

4. (a) The test specimen shall not be larger than No. 20 A. W. G. nor smaller than No. 22 A. W. G. The length of wire selected for tests shall be such as to permit the use of a 12" test length between the two terminals.

*Mounting of specimens*

5. (a) The test specimen shall be mounted on the test board in a vertical position and shall be spaced as follows:

|                                                | Inches |
|------------------------------------------------|--------|
| Distance between test board and specimens      | 2      |
| Distance between specimens                     | 6      |
| Distance between specimen and shield           | 2      |
| Distance between upper bus bar and mercury cup | 20     |

*Temperature of test*

7. The temperature of test shall be specified and shall be chosen so as to give a test life of approximately 100 hrs.

*Procedure*

8. The procedure shall be carried out as described in paragraphs (a) to (m), inclusive.

The results of the life test in relation to the calcium silicon addition to each melt were as follows:

|   | Manganese boron content grams (20% B) | MnB percent | Percent boron | CaSi, grams | CaSi, percent | Percent Ca | Percent Si added from CaSi | Percent Si added as Si | Total percent Si | Life, hours |
|---|---------------------------------------|-------------|---------------|-------------|---------------|------------|----------------------------|------------------------|------------------|-------------|
| 1 | 50                                    | .085        | .017          | 150         | .25           | .080       | .17                        | .66                    | .83              | 92          |
| 2 | 50                                    | .085        | .017          | 160         | .27           | .086       | .18                        | .66                    | .84              | 116         |
| 3 | 50                                    | .085        | .017          | 175         | .30           | .097       | .20                        | .66                    | .86              | 155         |
| 4 | 50                                    | .085        | .017          | 190         | .32           | .102       | .22                        | .66                    | .88              | 188         |
| 5 | 50                                    | .085        | .017          | 250         | .42           | .134       | .28                        | .66                    | .94              | 246         |

I have additionally discovered that controlled residual quantities of zirconium in conjunction with calcium silicon, when present in an alloy containing nickel, chromium and boron will result in a highly improved life characteristic. For example, employing the same test method as previously outlined, on nickel-chromium alloys containing the indicated amounts of boron, zirconium and calcium silicon, life tests of 264 and 149 hours were obtained in products which could be readily worked by conventional methods.

| Manganese boron content in grams | Percent boron | Silicon zirconium in grams | Percent silicon zirconium | Calcium silicon in grams | Percent calcium silicon | Life of specimen in hours |
|----------------------------------|---------------|----------------------------|---------------------------|--------------------------|-------------------------|---------------------------|
| 57<br>38                         | 0.10<br>0.06  | 50<br>100                  | 0.09<br>0.17              | 150<br>150               | 0.25<br>0.25            | 264<br>149                |

Thus the life imparting characteristics of zirconium may be extended through a range which would be unworkable without the addition of boron.

In compounding the above enumerated alloys, I found that more satisfactory results are obtained by using the calcium and zirconium diluents in the form of alloys or compounds of silicon because of their greater stability in this form. In this connection, it will be understood that direct additions of calcium and zirconium would entail relatively high losses from oxidation. Furthermore, calcium and zirconium are readily obtainable commercially in the form of com-

pounds of silicon. These commercial forms of calcium and zirconium contain relatively large percentages of silicon and some iron, as will be apparent in the following typical analysis of typical commercial samples of the products.

|                   | Ca         | Si         | Fe          | Zr         |
|-------------------|------------|------------|-------------|------------|
| Calcium silicon   | Percent 33 | Percent 62 | Percent 2.5 | Percent 36 |
| Silicon zirconium |            | 50         | 10.0        |            |

In the accompanying chart I have graphically illustrated the influence of boron in combination with a life-imparting diluent upon the factors of workability and increased life in the finished product.

More particularly, it will be seen that the grams calcium silicon content have been set off as abscissae, ranging from a minimum of 150 grams to a maximum of 250 grams. The life characteristics of alloys containing the previously mentioned proportions of calcium silicon have been set off as ordinates.

The curve C represents the result of the tests of boron and calcium silicon containing specimens above set forth. Thus, the point 1 represents a calcium silicon content of 150 grams

which, in conjunction with 50 grams of manganese boron, provided a life test of 92 hours.

The point 2 corresponds with the second test specimen in which the calcium silicon content was 160 grams and the life test 116 hours.

Point 3 corresponds with the third test specimen in which 175 grams of calcium silicon provided a life test of 155 hours.

Correspondingly, points 4 and 5 are predicated upon the specimen similarly numbered in the first table.

Now it will be seen that the curve C is developed by connecting the points 1, 2, 3, 4 and 5 with the smooth projection.

I have found that a calcium silicon content in excess of 160 grams, or 0.27% without the presence of boron, makes for an unworkable product. Thus it may be said that point 2 on the curve C is representative of the limits of workability, and consequently the optimum quantity of life-imparting diluent which can be added to the basic alloy without the additional presence of boron.

Examining the curve further, it will be apparent that boron renders the product workable and thus usable and practicable in a commercial sense with calcium silicon content in excess of 0.27%.

Otherwise stated, the practicable limit of increase in life-imparting diluents has been elevated from 0.27% to 0.42%. This has been shown by the production of workable materials containing these higher calcium silicon contents and reflected in the increase in life by the standard tests from 116 to 346 hours.

It will be obvious that life tests in excess of 116 hours could not be obtained were it impracticable to manufacture wire to be subjected to the test.

I claim as my invention:

1. A nickel chromium alloy containing 0.34% of a metal of the alkaline earth group, approximately 0.01% of boron, approximately 20% of chromium, the balance nickel.
2. A nickel chromium alloy containing 0.25% to 0.42% of calcium, approximately 0.02% of boron, approximately 20% of chromium and the balance nickel.

3. A nickel chromium alloy containing approximately 0.27% of calcium, approximately 0.02% of boron, approximately 20% of chromium, and the balance nickel.
4. A non-ferrous metal alloy containing nickel approximately 80%, chromium approximately 20%, a metal of the alkaline earth group from substantially 0.27% to 0.42% and boron from 0.02% to 0.01%.

ERICH FETZ.